

## UNITED STATES PATENT OFFICE.

EDMUND VON HERZ, OF BERLIN-CHARLOTTENBURG, GERMANY.

## METHOD OF MANUFACTURING DETONATING COMPOSITIONS FOR EXPLOSIVE AND PERCUSSION CAPS.

No Drawing. Application filed October 21, 1925, Serial No. 64,054, and in Germany October 23, 1924.

The numerous substitutes recently suggested for fulminate of mercury and lead azide in explosive and percussion caps are not regarded for certain reasons as completely equivalent substitutes for these two excellent igniting agents.

It has now been discovered that the metallic salts of the iso-nitro-amines which are also named, nitroso-hydroxyl-amines or di-nitrosyl acids constitute exceptionally good substitutes for these two primings.

It will be noted that these three names are used in the literature to designate a single group of chemical compounds. The general structural formula of the group of compounds is



whereas the structural formula of the real nitramines is



and



The most important representatives of these iso-nitro-amines, and substances which are also most suitable for the present purpose, are methylene di-iso-nitro-amine, ethylidene di-iso-nitro-amine, the iso-nitro-amine fatty acids and the iso-nitro-amine derivatives of the nitro-paraffins. All these substances are obtained in good yields by treating the associated ketones and nitro-paraffins in alcoholic solution in the presence of sodium ethylate with oxide of nitrogen (see "Annalen der Chemie," 300, page 81).

Thus methylene di-iso-nitro-amine is produced from acetone by this reaction. The feebly explosive sodium salts resulting from this process are converted in a known manner into salts of heavy metals, of which especially the lead salts, not only the neutral but also the monobasic and polybasic lead salts, are valuable for this purpose.

While the free iso-nitro-amine compounds decompose with extreme readiness, the salts are characterized by great stability, which renders them particularly suitable for the present purpose.

The behavior of the most important of these salts, the lead salt of methylene di-iso-nitro-amine, is very peculiar from the point

of view of explosive technology. Ignited in free air, it burns with only a slight explosion. When pressed into a detonator case it only hisses out or explodes with only quite a feeble effect. The speed of libration of the detonation is therefore only small. If however some lead tri-nitro-resorcinate is added, whether as a loading or as an admixture, the salt detonates with excellent effect. An addition of salts of hexa-nitro-di-resorcinal, tri-nitro-phloro-glucinol, hexa-nitro-di-phenyl amine, di-nitro-di-nitroso-benzene, basic nitro-body salts such as monobasic and polybasic lead picrate phenolate and di-nitro-phenolate and salts of similar nitro-bodies, acts in a similar manner. The lead salt of methylene di-iso-nitro-amine is thus in a sense exploded by these comparatively feebly acting salts. Of course mercury fulminate and lead azide may also be employed for this purpose, but this obviously presents no advantage.

The salts of the remaining iso-nitro-amines behave just in the same way; but the capacity, owing to the more unfavorable oxygen balance, is not quite so good.

For practical use there come into consideration firstly the lead salt of methylene di-iso-nitro-amine, the structural formula of which is:



and secondly that of ethylidene di-iso-nitro-amine the structural formula of which is:



It is advantageous to employ these two substances together, as they are complementary to one another as regards their oxygen content.

The construction of a detonating cap on this basis would be carried out either by placing in the detonator case on top of a certain quantity of these lead salts about 0.1 gr. of lead tri-nitro-resorcinate or of the other bodies, or by utilizing a unitary charge of a mixture with from 50 to 25 per cent. of the said bodies. Obviously the detonating caps can also be manufactured to the combination principle, from 0.3 to 0.4 gr. of the iso-nitro-amine salts and then about 0.1 gr. of the said nitro-body salts for example be-

ing placed on top of the secondary tetryl or tri-nitro-toluol charge, or even more advantageously by employing a priming top consisting of mixtures of the iso-nitro-amine salts with the nitro-compound salts, for example 0.4 gr. of a 50 to 75 per cent. mixture of lead methylene di-iso-nitro-amine with lead tri-nitro-resorcinate. Even more effective than mere mechanical mixtures are mixed salts obtained either by joint, simultaneous precipitation of the iso-nitro-amine salts with the nitro-compound salts or precipitation of one of the components upon the other already precipitated and suspended in the precipitant. In consequence of the uniform distribution and intimate mixing of the components in these mixed salts, which in part represent definite complex compounds, the speed of the explosive conversion and consequently also the priming or exploding power is considerably greater and the latter surpasses in many cases that of mercuric fulminate. The limiting charges of a 70 and 30 per cent. mixed salt of lead methylene di-iso-nitro-amine and lead tri-nitro-resorcinate are for example 0.09 gr. for tetryl and 0.15 gr. for tri-nitro-toluol. Since all these salts possess a good sensitivity to percussion, without however being over-sensitive, they are exceedingly suitable for the manufacture of priming or detonating compositions for percussion caps, especially as they also have a good priming power. In this case the salts are employed in the usual way by themselves or in connection with the usual components of priming compositions, preferably also in common with the salts of nitro compounds, especially in the form of jointly precipitated mixed salts.

The main advantage of these new salts lies in the remarkably easy accessibility and the consequent low price of these salts.

What I claim is:—

1. A process for the manufacture of priming compositions for detonators and percussion caps, comprising the employment of the metallic salts of the iso-nitro-amines. 45
2. A process for the manufacture of priming compositions for detonators and percussion caps, comprising the employment of the metallic salts of the iso-nitro-amines, in conjunction with other priming compositions. 50
3. A process for the manufacture of priming compositions for detonators and percussion caps, comprising the employment of the metallic salts of the iso-nitro-amines, in conjunction with other explosives. 55
4. A process for the manufacture of priming compositions for detonators and percussion caps, comprising the employment of the metallic salts of the iso-nitro-amines, in conjunction with other components of priming compositions. 60
5. A process for the manufacture of priming compositions for detonators and percussion caps, comprising the employment of the metallic salts of the iso-nitro-amines, in conjunction with lead tri-nitro-resorcinate. 65
6. A process for the manufacture of priming compositions for detonators and percussion caps, comprising the employment of the metallic salts of the iso-nitro-amines, in conjunction with such salts of nitro compounds which are equivalent in force and igniting power to the lead trinitroresorcinate. 70

In testimony whereof I have signed my name to this specification.

EDMUND VON HERZ.